

3 Sheets—Sheet 1.

H. BLACKMAN.

## DISINTEGRATING FIBERS AND MANUFACTURING PAPER PULP.

No. 369,836.

Patented Sept. 13, 1887.



Witnesses  
John H. Smith  
I. Stahl

Henry Blackman  
for Samuel M. Ferrell

(No Model.)

H. BLACKMAN.

3 Sheets—Sheet 2.

DISINTEGRATING FIBERS AND MANUFACTURING PAPER PULP.

No. 369,836.

Patented Sept. 13, 1887.



Witnesses

Chas H. Smith  
J. Stahl

Inventor

Henry Blackman  
for Samuel W. Ferrell  
a.m.

(No Model.)

3 Sheets—Sheet 3.

H. BLACKMAN.

DISINTEGRATING FIBERS AND MANUFACTURING PAPER PULP.

No. 369,836.

Patented Sept. 13, 1887.



Fig. 5.

WITNESSES :

Arthur Wilson.

George Müller

INVENTOR :

Henry Blackman.  
By his Attorneys.

Arthur C. Fraser & Co.

# UNITED STATES PATENT OFFICE.

HENRY BLACKMAN, OF NEW YORK, N. Y.

## DISINTEGRATING FIBERS AND MANUFACTURING PAPER-PULP.

SPECIFICATION forming part of Letters Patent No. 369,836, dated September 13, 1887.

Application filed May 17, 1886. Renewed August 5, 1887. Serial No. 246,208. (No model.)

To all whom it may concern:

Be it known that I, HENRY BLACKMAN, a citizen of the United States, residing in the city, county, and State of New York, have invented certain new and useful Improvements in Disintegrating Fibers and Manufacturing Paper-Pulp, of which the following is a specification.

My invention relates to the manufacture of paper-pulp from wood, straw, jute, or other fibrous substances.

Prior to my invention fibers have been disintegrated by boiling them under pressure in a closed vessel, usually with an alkali or other chemical, and when sufficiently softened by this treatment opening the outlet of the vessel and discharging its contents suddenly into the atmosphere. During this discharge the over-heated liquid in the cells or interspaces between the fibers, being relieved of pressure, suddenly vaporizes and expands, tearing the fibers asunder. This method of "exploding" the fibrous substances is objectionable in many respects, among others the scattering of the fibrous matter in all directions and the large space required.

My invention provides a method of disintegration based upon the same principle, which is designed to overcome the difficulties heretofore encountered.

My invention relates both to the method of treatment and to the apparatus for practicing that method.

According to my invention the fibrous substance to be reduced to pulp is placed in a closed digesting-vessel and exposed to the action of water, with or without other chemicals, and under more or less pressure, until the material is sufficiently dissolved or softened. This done, the material, being at the time charged with fluid under heavy pressure, is forced out from the digester through a contracted nozzle or inlet-opening, which enters a vacuum-chamber, and the material as it escapes from the nozzle into this chamber is disrupted by the sudden expansion or explosion of the fluid (steam or superheated water) in the interstices of the fibers. The explosive action is more effective by occurring in a partial vacuum, and this vacuum is maintained by the continuous action of an air-pump or other suitable exhausting device. The de-

struction of the vacuum by the expansion of the steam in the vacuum-chamber is prevented by the nozzle, which is so contracted that it retards the admission of fibrous material and liquid, admitting it in so reduced a stream that the steam therefrom is of no greater volume than the capacity of the pump will suffice to draw off. To quickly reduce the volume of the steam after its expansion and assist in maintaining the vacuum, the chamber is continually cooled after the manner of a condenser, preferably by showering cold water into it through jet-pipes. This water minglest with the disrupted fibrous material, and the whole is drawn off and subjected to further treatment.

In order to thoroughly separate the fibers and reduce the entire fibrous mass to a uniform condition, I pump the same, with water, through a long tortuous passage—as a coil of pipe—wherein obstructions are provided to agitate the fibers. When this action is completed, the diluted fibrous matter or pulp is washed through a series of traps or separators, by which the hard particles and grit are arrested. The pulp is then flowed over screens and sprinkled with jets of water to wash and screen out the coarser particles.

The accompanying drawings show the apparatus constructed according to my invention and used for practicing my improved process.

Figure 1 is a vertical section of the digester and vacuum-chamber and an elevation of the coil and pump. Fig. 2 is a vertical section, and Fig. 3 a cross-section, of a fragment of the coil on a larger scale; and Fig. 4 is a vertical section showing a modification of portion of the apparatus. Fig. 5 is a vertical section showing a modification of the vacuum-chamber and exhauster.

In Fig. 1, A designates the digester, which is a strong closed vessel capable of withstanding a considerable pressure and of such material or lined with such material as will resist the action of the chemicals used. A steam-pipe, B, enters it, preferably from the top, and extends to or nearly to the bottom. There may also be another steam-pipe, B', entering the vessel and terminating near the middle thereof. A man-hole, C, is provided, preferably at the top, through which to introduce

the materials to be treated, and at the bottom is an outlet-cock, D. The bottom portion of the vessel should slope downward toward this outlet. I prefer to construct it with a conical strainer, a, sloping toward the outlet and forming an annular space, b, from which any chemicals or liquors may be drained off through a tap, c. The cock D opens into a pipe, E, which leads thence upward to a vacuum-chamber or condenser, F, which it enters, terminating in a contracted nozzle, e.

The fibrous matter to be disintegrated, being properly comminuted, is introduced into the digester through the man-hole C, and the 15 digester is closed. Water is introduced either with the material or separately, and either with or without any suitable chemical agents—such as alkali or sulphurous acid, or other substances, according to the chemical process 20 which is preferred. Steam is turned on and the mass is subjected to heat, with more or less pressure, (or, if preferred, without pressure, or even *in vacuo*), for a sufficient length of time and until the fibrous matter is properly dis- 25 solved or softened. When the mass is ready to be discharged, it is blown out through the pipe E into the vacuum-chamber F, where it is disrupted by the expansive action. The discharge is effected by opening the cock D, when 30 the pressure of steam within the digester forces out the pulp and water. If there is not sufficient pressure already in the digester, steam is to be admitted through the pipe B'. It is preferable to drain off through the tap c any chemicals 35 that have been used and reclaim them, introducing water in their place (if necessary) to dilute the semi-pulpy fibrous matter to the proper fluidity to enable it to flow properly; or the fibrous matter might be forced out by 40 the steam-pressure without adding water. In such case it is only essential that the fibrous matter shall have been sufficiently softened to be capable of disruption, that the fluid-pressure shall have penetrated its interstices, and 45 that there be sufficient pressure both to disrupt the fibers after passing the nozzle and to force the fibrous matter through the nozzle. The flow of the fibrous material and water through the pipe E is retarded by the nozzle 50 e, which holds back the stream, as it were, and admits only a comparatively small jet into the vacuum-chamber F. As the fibrous matter passes the nozzle and emerges into the 55 vacuum, it is suddenly relieved from pressure and the steam in the interstices of the fibers expands and tears them apart. This expansion is due, in a measure, to the vaporization of the water, which has been heated above the boiling-point but its ebullition suppressed by 60 the superincumbent pressure until its discharge at the nozzle. I provide in the pipe E a steam-jet pipe, d, adapted to discharge a jet of steam into the mass of fibrous material in order to increase its pressure by acting against 65 it on the principle of the injector. The steam enters through a pipe, f, and is controlled by a valve, g, the jet being regulated by a screw.

pin or cone, h, as is usual in boiler-injectors. This injector is chiefly useful when the pressure in the digester is too low to cause a sufficiently forcible disruptive action. It is also useful when there is any clogging in the pipe E. 70

The vacuum-chamber F is of any convenient shape and of suitable size. It is preferably divided into two compartments by a partition, 75 F', which serves as a shield or target to receive the impact of the fibrous matters projected from the nozzle. The harder particles—such as bits of knots—which are not blown apart by the expansion of the steam, are aided in 80 their disintegration by striking this target. The fibrous mass falls to the bottom of the chamber, whence it is washed under the partition and carried down the pipe F' to the pump F'. This pump is operated by a steam- 85 engine, G, or other source of power, and acts to draw the pulpy matter, water, and vapors from the chamber F, and to maintain a partial vacuum therein. Separate pumps may be used, if preferred, for the liquids and vapors; 90 but one will serve for both.

The maintenance of the vacuum is materially facilitated by showering water into the chamber F, which acts to condense the steam therein. A perforated pipe, P P', enters the 95 chamber and receives water under pressure, which it discharges into both compartments in jets. This water mingles with the pulp and further liquefies it. A surface-condenser might be used in place of a jet-condenser, if 100 desired; but I prefer the latter.

The capacity of the pump F' must be such that with a given pressure upon the entering pulp and water and a given area of nozzle, and with a given condensation due to the showering of water, the suction of the pump will draw off the vapors from the vacuum-chamber faster than they enter it, in order to maintain a sufficient vacuum therein. I prefer a vacuum of about twenty-seven inches; but 110 this may vary. Even a slight rarefaction, sufficient to draw off the vapors as fast as they enter, so as to afford a free space to receive the entering pulp, water, and steam from the nozzle, is of great advantage, as otherwise a 115 pressure would soon accumulate in the chamber F, (even if it were provided with escape-openings for the steam,) which would materially reduce the effectiveness of the disruptive action in tearing apart the fibers. 120

In place of the pump F', any other suitable device may be employed for exhausting the vapors from the chamber F—as an injector, for example, as will be presently described.

From the pump the pulp and water is 125 forced through an extended and preferably tortuous passage, in which are agitating obstructions. The coil R R of pipe affords the extended passage, in passing through which the pulp flows up and down, being agitated by 130 the bubbling through it of the steam and gases, and by contact with suitable mechanical obstructions against which the liquid flows, thereby gently rubbing the fibers and

promoting their separation. This method of agitating the pulp and separating the fibers I do not claim of itself in this application, but shall make it broadly the subject of another 5 application for patent to be filed by me.

Figs. 2 and 3 show the obstructions in the coil R, consisting of wire helices N N, preferably three in number, arranged triangularly. The coil R terminates in the first of a series 10 of precipitating vessels or troughs, S' S' S'. Dipping into these vessels are partitions 3, 4, and 5, and between them are dams 6, 7, and 8. The pulp and water entering the upper vessel flows down under the partition 3 and up over the dam 6 into the second vessel. There may be any number of vessels, and in 15 each the liquid flows downward under a partition and then upward over a dam. As it flows downward, its heavier particles are directed toward the bottom, where they fall and lie undisturbed by the current above them. In this manner any particles of sand, grit, or other heavy foreign bodies are removed 20 from the pulp. The pulp flows from the lower vessel onto an inclined screen, S, where it is 25 sprinkled or showered with water from pipes I I. The pulp is thus washed through the meshes of the screen; but any coarse particles are arrested and retained on the screen. Beneath this screen is another screen, T, of 30 finer mesh, on which the pulp is again rinsed or showered with water from pipes J J. The fine pulp passes through this screen and falls on an inclined endless apron, Q, of muslin or 35 other fine fabric, turning over rollers 25 26. The water flows through the fabric, leaving the fibrous matter on the apron, whence as the apron revolves it is delivered at the roller 26. A sprinkler, K, may be used to still further 40 wash the pulp on the apron. Any other desired method of delivering the pulp or fibrous matter may be used instead of that here shown.

Fig. 4 shows a modified construction of screens for washing the pulp. From the vessel S' the pulp flows upon an endless screen, S, of wire-cloth, which is carried around rollers 13 13. An inclined plate, 23, receives the pulp as it is washed through the screen S, and carries it onto a second endless screen, T, of 50 wire-cloth of finer mesh. An inclined plate, 19, receives the pulp which passes through the screen T and directs it onto the apron Q, where the water is drained off and the pulp is delivered over the roller 26. The screens S T 55 are caused to revolve, and the coarse particles separated from the pulp are dropped off at their ends or are washed off from the under sides.

In Fig. 5 a modification of my apparatus is 60 illustrated, wherein the suction-pump F<sup>3</sup> is omitted and an injector substituted. The digester A, steam-pipes B B', valve D, steam-injector f g h d, and outlet-pipe E are all of substantially the same construction already 65 described. In place of the pump F<sup>3</sup> for exhausting the vapors, there is a hydraulic injector or ejector, F<sup>4</sup>, connected to the vacuum-

70 chamber. This ejector employs a column of water under pressure, which passes through a nozzle in such manner as to produce a powerful suction around the nozzle in a space or chamber which communicates with the vacuum-chamber. The water under pressure is supplied through a pipe, i, and enters the nozzle H, being controlled by a valve, j, which 75 is adjustable vertically by a screw, k, in order to close the nozzle H more or less. The column of water issuing rapidly from the nozzle H passes downwardly into a flaring tube, m. A chamber, K, surrounds the nozzle, and is 80 connected by a tube, O, with the vacuum-chamber F, so that the suction produced by the water acts to exhaust the vapors from the chamber F and maintain the partial vacuum therein. The water flows off through the pipe 85 L, carrying with it any fibers that may have been drawn off with the vapors, these fibers being recovered by means of a sieve. This ejector device for exhausting the vacuum-chamber is not recommended as a substitute 90 for the pump, but may be used to advantage in some situations where there is an abundance of water at an elevated head.

In place of using a large pipe, E, terminating in a contracted nozzle, the pipe may be 95 made as small as the nozzle throughout its entire length, in which case the end of the pipe where it entered the chamber F would constitute in effect a nozzle. By the term "nozzle" I mean the inlet to the vacuum-chamber, and by "contracted nozzle" I mean such an inlet which is contracted relatively to the pressure, the rapidity of condensation, and the capacity 100 of the pump, so that it admits the pulp and water no faster than the vacuum can be maintained. The pipe E may be of greater or less length, and the vacuum-chamber may be arranged at any desired height. If preferred, 105 the vacuum-chamber may be arranged low down and the pipe E be made very short. 110

I claim as my invention—

1. The improvement in the art of disintegrating fibrous substances, which consists in charging them with fluid under pressure and at a high temperature and forcing them in a 115 reduced stream into a partial vacuum, whereby the expansion of the fluid when liberated in the vacuum disrupts the fibers.

2. The improvement in the art of disintegrating fibrous substances, which consists in softening the fibers by digesting them in a closed vessel, charging the softened fibers with fluid under pressure and at a high temperature, and forcing them through a contracted nozzle or inlet into a partial vacuum, whereby 125 the expansion of the fluid when liberated in the vacuum disrupts the fibers.

3. The improvement in the art of disintegrating fibrous substances, which consists in softening the fibers by chemical treatment, 130 charging the softened fibers with fluid under pressure and at a high temperature, and forcing them through a contracted nozzle or inlet into a partial vacuum.

4. The improvement in the art of disintegrating fibrous substances, which consists in softening the same by treatment with liquid in a closed digester, charging the softened fibers with liquid under pressure and at a high temperature, and forcing the fibers and liquid through a contracted nozzle or inlet into a vacuum-chamber. 65
5. The improvement in the art of disintegrating fibrous substances, which consists in charging the fibers with fluid under pressure and at a high temperature, forcing them through a contracted nozzle or inlet into a vacuum-chamber, and continually drawing off the contents of said chamber at a rate sufficient to prevent the accumulation of a pressure therein. 7c
10. The improvement in the art of disintegrating fibrous substances, which consists in forcing the same with liquid under heat and pressure through a contracted nozzle or inlet into a vacuum-chamber, condensing the steam therein, and drawing off the contents of said chamber at a rate sufficient to maintain a partial vacuum therein. 75
15. The improvement in the manufacture of paper-pulp, which consists in first softening a fibrous substance by treatment with liquid, then disrupting the fibers by liberating them under heat and pressure in a closed chamber, and then forcing the fibers with water through an extended passage containing agitating obstructions, whereby the fibers are separated. 80
20. The improvement in the manufacture of paper-pulp, which consists in first softening a fibrous substance by treatment with liquid, then disrupting the fibers by liberating them under heat and pressure in a closed chamber, and subsequently separating the heavier particles by precipitation from the fluid pulp. 85
25. The improvement in the manufacture of paper-pulp, which consists in first softening a fibrous substance by treatment with liquid, then disrupting the fibers by liberating them under heat and pressure in a closed chamber, and finally washing the pulp through screens to remove the coarser particles. 90
30. The improvement in the manufacture of paper-pulp, which consists of the following succession of steps: first, softening the fibrous substance by treatment with liquid; second, disrupting the fibers by liberating them under heat and pressure in a closed chamber; third, forcing the fibers with water through an extended passage containing agitating obstructions; fourth, separating the heavier foreign particles by precipitation, and, fifth, separating the coarser particles by washing through screens. 95
35. 11. An apparatus for disintegrating fibrous substances, consisting of the combination of a digester, a vacuum-chamber, an outlet-passage from the digester to said chamber, and a valve in said passage, substantially as set forth. 100
12. The combination of a digester, a vacuum-chamber, an outlet-passage from the digester to said chamber, a valve in said passage, and an exhausting apparatus connected to said chamber and adapted to maintain a vacuum therein, substantially as set forth. 105
13. The combination of a digester, a vacuum-chamber, an outlet-passage from the digester to said chamber, a valve in said passage, and a condenser arranged and adapted to condense the steam in said chamber, substantially as set forth. 7c
14. The combination of a digester, a vacuum-chamber, an outlet-valve to the digester, a discharge pipe or passage leading thence to said chamber, and a steam-jet pipe or injector in said passage, substantially as set forth. 110
15. The combination of a digester, a vacuum-chamber, an outlet-passage from said digester to said chamber, a contracted nozzle terminating said passage and entering said chamber, and a pump with its exhaust connected to said chamber, substantially as set forth. 115
16. The combination of a digester, a vacuum-chamber, a valved passage connecting them, a pump connected to said chamber, and a coil of pipe through which the pulp and water are discharged and in which the fibers are subjected to agitation, as described. 90
17. The coil of pipe for agitating the fibers, having within the same helices of metal, in combination with a pump to force the pulp through the coil and helices, substantially as set forth. 120
18. In a pulp-making apparatus, a separator for precipitating heavy particles, consisting of a succession of vessels provided with alternate downwardly-projecting partitions under which the liquid must flow and dams over which it must flow, substantially as set forth. 105
19. The combination of the pump, the agitating-coil, and the separator for precipitating the heavier particles, receiving the pulp as it leaves said coil, substantially as set forth. 110
20. In a pulp-making apparatus, a screening device for separating coarse particles, consisting of one or more fine screens over which the pulp is flowed, with sprinklers arranged to shower water thereon, and an endless traveling apron receiving the pulp as it passes through said screen and adapted to drain it of water, substantially as set forth. 115

Signed by me this 11th day of May, A. D. 1886.

HENRY BLACKMAN.

Witnesses:

GEO. T. PINCKNEY,  
WILLIAM G. MOTT.